# EUROPEAN PATENT SPECIFICATION

(11) **EP 0 500 854 B1**
(45) Date of publication and mention of the grant of the patent: **04.01.1995**
(21) Application number: 91915315.5
(22) Date of filing: 03.09.1991
(51) Int. Cl.: C23C 4/06, C23C 4/18, C23C 4/12, F01D 5/28, F01D 25/00

(54) **A COATING, AND A COATING METHOD, FOR A STEAM TURBINE AND ADJOINING STEEL SURFACES**
BESCHICHTUNG UND BESCHICHTUNGSVERFAHREN FÜR DAMPFTURBINEN UND BENACHBARTE STAHLOBERFLÄCHEN
REVETEMENT, PROCEDE DE REVETEMENT POUR TURBINE A VAPEUR ET SURFACES D'ACIER CONTIGUES

(30) Priority: 04.09.1990 FI 904369
(43) Date of publication of application: 02.09.1992
(73) Proprietor: TELATEK OY, SF-92100 Raahe (FI)
(72) Inventor: TENKULA, Jaakko, SF-92120 Raahe (FI); HELLMAN, Bjarne, SF-11910 Riihimäki (FI); MAJAVA, Jorma, SF-11120 Riihimäki (FI)
(74) Representative: UEXKÜLL & STOLBERG
(86) International application number: FI9100269
(87) International publication number: WO9204480

(56) References cited:
- GB-A- 1 439 947
- GB-A- 1 448 256

## Description

The invention relates to a coating intended for protecting the interior surfaces of a steam turbine and the adjoining pipes and superheaters, the coating preventing the erosive and corrosive wear caused by steam. The invention also relates to a method for coating the interior surfaces of a steam turbine and the adjoining pipes and superheaters.

As stated in Swedish Patents/Patent Applications No. 762881 and 771073, steel surfaces exposed to hot, damp steam at high pressures and velocities are subject to heavy erosive and corrosive wear.

The damage caused by wear may lead to the need for fill-in and repair weldings which are difficult to carry out, and even replacement of the turbine casing and pipes.

Such repair and replacement work causes long stoppages and thereby large financial losses owing to reduced production. This is the case in particular in large power plants such as nuclear power plants.

For example the following coatings have been used for protecting turbine pipes:
1. Ceramic coating with a nickel-aluminum alloy in the adhesive layer. The thickness of the adhesive layer is 10 - 25 µm and that of the ceramic coating 50 - 250 µm.
2. Metallic so-called triple-layer coating, in which the adhesive layer is a nickel-aluminum alloy (t = 50 - 100 µm), the intermediate layer is a chromium steel (approx. 13 % Cr, with a layer thickness of approx. 200 µm), and the surface layer is a stainless or acid-resistant steel (Cr = approx. 18 %, Ni = 5 - 8 %, and Mn = approx. 8 %, with a layer thickness of approx. 200 µm).

Ceramic coatings have, for example, the following disadvantages:
- poor shock resistance, for example, when foreign bodies enter the turbine or the pipes, they may break the coating;
- the thermal expansion coefficient of a ceramic coating is very low compared with that of carbon steel, so that great or rapid variations in the temperature may lead to the cracking of the coating. A crack in the coating may, in turn, lead to rapid local damage to the base material;
- ceramic coatings are good insulators. The coating of a turbine casing with a ceramic material could disturb intra-turbine thermal conduction and cause unexpected deformation during operation;
- with a ceramic coating it is difficult to coat seal surfaces which are to be machined. The coating may have a hardness higher than 1000 HV, and therefore it is difficult to machine, and, furthermore, the coating tends to crack;
- it is difficult to achieve a sufficient layer thickness with a ceramic coating if the coating is to be used for filling cavities.

So-called triple-layer coating has functioned satisfactorily in pipe systems. However, this coating has the following disadvantages:
- in a triple-layer coating, each interface between the different coatings constitutes a strong barrier to thermal conduction, and so problems similar to those involved with ceramic coatings may appear in thermal conduction in the turbine casing;
- if it is necessary to fill cavities in coating surfaces which are to be machined, there is the risk that the machines surface will run through different layers;
- if the triple-layer coating is damaged in operation, for example owing to strong local erosion, it must be repaired by first removing the old coating entirely and by then recoating the surface, layer by layer.

The primary object of the present invention is to provide a coating which can be used for coating the casing, division planes, piping, superheaters and other parts of a steam turbine so that reliable and long-term protection, suitable for the conditions involved, is obtained for the steel surfaces. It is a further object of the invention that the coating work can be carried out on the site rapidly and economically, and that the coating is also well suited for the coating of surfaces which are to be machined.

The coating on a steel part according to the invention is characterized in that the coating comprises a coating layer which is obtainable by the thermal spraying of a steel alloyed with chromium and aluminum in the below stated amounts, which, during the coating process, oxidize in the spray, whereby chromium and aluminum oxides are formed which will remain inside the coating, surrounded by a steel matrix, and on the surface of the coating layer there will form, after the coating process, under the oxidizing effect of air, a dense chromium and aluminum oxide film.

The coating method according to the invention is characterized in that a coating material of steel alloyed with chromium and aluminum in the below stated amounts is sprayed thermally onto the surface being coated, and this coating material oxidizes in the spray during the coating process, whereby chromium and aluminum oxides are formed which will remain inside the coating, surrounded by a steel matrix, and that, after the coating process, the coating which has been formed will be exposed to the oxidizing effect of air, whereby a dense chromium and aluminum oxide film will be formed on the surface of the coating.

According to the invention, the coating material used is a steel containing chromium 20 - 45 % by weight, aluminum 5 - 15 % by weight and molybdenum 0 - 5 % by weight, and especially preferably chromium 22 - 30 % by weight, aluminum 5 - 8 % by weight and molybdenum 0 - 3 % by weight. The coating material may be thread-like or pulverous.

The chromium and aluminum oxide film in the coating according to the invention, formed under the effect of oxidation after the coating process, is strong and dense, and will prevent erosive and corrosive wear caused by wet steam.

The coating according to the invention can be prepared by thermal spraying, by using flame, arc, plasma and/or supersonic spraying, but primarily arc, plasma and/or supersonic spraying, in order to obtain good adhesion of the coating to the base material.

Thus there is formed in the coating according to the invention a layer with good adhesion to the base material, a steel coating which contains a large amount of oxides, and a surface layer which consists of a dense oxide film.

In order that no galvanic corrosion should occur on the interface between the base material and the coating, the thickness of the coating should be at minimum 0.3 mm, preferably, however, 0.5 mm. The thickness of the coating may be up to 2.5 mm without its pealing off because of internal shrinkage of the coating.

The advantages of the coating according to the invention as compared with previous ones are as follows:
1. The very dense chromium and aluminum oxide film formed on the surface of the coating provides excellent protection against corrosion and erosion. Nevertheless, the coating is very tough.
   If the coated surface is damaged, for example under the effect of a foreign body which has entered the turbine, the oxides inside the coating will prevent propagation of the damage.
   Thus the coating provides the protective effect of a ceramic coating, but it has the toughness and strength of a metal coating.
2. The adhesion of the coating to the base material is very good. When arc or plasma spraying is used, an adhesion strength greater than 60 N/mm is obtained, which is approximately double the adhesion strength of a flame-sprayed nickel and aluminum alloy.
   Good adhesion guarantees that the coating will not become detached by minor impacts, and that it will also be possible to coat narrow edges. Furthermore, good adhesion enables the surface to be machined.
3. The thermal expansion coefficient of the coating is close to the thermal expansion coefficient of carbon steel, so that deformation due to thermal shock and thermal expansion will not damage the coating.
4. Since the coating is made up of one single layer and it can be sprayed approx. 2 mm thick, the coating is suitable for protecting very large seal surfaces which are to be machined.
5. Although the coating contains large amounts of hard oxides, its macro-hardness is only 250 - 350 HV units, so that the coating will be easy to machine.
6. Thermal conduction will not cause problems, since the only interface hampering thermal conduction is the interface between the coating and the base material.
7. Patching of the coating is easy to perform locally, without removing all of the old coating.
8. The cobalt content of the coating is very low (approx. 0.02 %), and so the coating is highly suitable for use in nuclear power plants, also on surfaces on the active side.
   In a nuclear power plant the division planes and some of the turbine casing above and below the division planes were coated by arc spraying with a coating according to the invention, the analysis of which was 22 % Cr and 5 % Al.
   After eight years of use the turbine was opened, whereupon it was observed that the division planes were completely flawless and that the coating above and below the division planes had endured very well. On the other hand, the base material had worn off up to more than 10 mm in the area adjacent to the border of the coating.

## Claims

1. A coating on a steel part useful for protecting the casing, division planes, piping, superheaters and other steel parts of a steam turbine which are subjected in a turbine plant to some corrosive and erosive wear caused by hot wet steam, which is obtainable by thermally spraying a steel alloyed with 20 to 45 and preferably 22 to 30% by weight of chromium, 5 to 15 and preferably 5 to 8% by weight of aluminum and 0 to 5 and preferably 0 to 3% by weight of molybdenum onto the surface of the part to be coated, the chromium and aluminum oxidizing in the spray during the coating process, whereby chromium and aluminum oxides are formed which will remain inside the coating, surrounded by a steel matrix, and by exposing the surface of the so formed coating layer to the oxidising effect of air to form a dense chromium and aluminum oxide film.

2. A coating according to Claim 1 consisting of one layer with a thickness of 0.3 to 2.5 mm.

3. A method for coating the casing, division planes, piping, superheaters and other steel parts of a steam turbine which are subjected in a turbine plant to some corrosive and erosive wear caused by hot wet steam, in which a steel alloyed with 20 to 45 and preferably 22 to 30% by weight of chromium, 5 to 15 and preferably 5 to 8% by weight of aluminum and 0 to 5 and preferably 0 to 3% by weight of molybdenum in thermally sprayed onto the surface of the part to be coated, the chromium and aluminum oxidizing in the spray during the coating process, whereby chromium and aluminum oxides are formed which will remain inside the coating, surrounded by a steel matrix, and in which the surface of the so formed coating layer is exposed to the oxidizing effect of air to form a dense chromium and aluminum oxide film.

4. A method according to Claim 3 in which one layer with a thickness of 0.3 to 2.5 mm is formed.

5. A method according to Claim 3 or 4 in which the thermal spraying is carried out by the arc, plasma or supersonic method.

## Patentansprüche

1. Beschichtung auf einem Stahlteil, die zum Schutz des Gehäuses, der Trennebenen, der Rohrleitungen, der Überhitzer und anderer Stahlteile einer Dampfturbine, welche in einer Turbinenanlage einem durch heißen Naßdampf verursachten korrosiven und erosiven Verschleiß unterworfen sind, brauchbar und erhältlich ist, indem ein mit 20 bis 45 und vorzugsweise 22 bis 30 Gew.% Chrom, 5 bis 15 und vorzugsweise 5 bis 8 Gew.% Aluminium und 0 bis 5 und vorzugsweise 0 bis 3 Gew.% Molybdän legierter Stahl thermisch auf die Oberfläche des zu beschichtenden Teils gespritzt wird, wobei das Chrom und Aluminium während des Beschichtungsverfahrens in der Spritzmasse (dem Spray) oxidieren, wodurch Chrom- und Aluminiumoxide gebildet werden, die von einer Stahlmatrix umgeben im Inneren der Beschichtung verbleiben, und die Oberfläche der so gebildeten Beschichtungsschicht der Oxidationswirkung der Luft ausgesetzt wird, um einen dichten Chrom- und Aluminiumoxidfilm zu bilden.

2. Beschichtung nach Anspruch 1, die aus einer Schicht mit einer Dicke von 0,3 bis 2,5 mm besteht.

3. Verfahren zum Beschichten des Gehäuses, der Trennebenen, der Rohrleitungen, der Überhitzer und anderer Stahlteile einer Dampfturbine, welche in einer Turbinenanlage einem durch heißen Naßdampf verursachten korrosiven und erosiven Verschleiß unterworfen sind, bei dem ein mit 20 bis 45 und vorzugsweise 22 bis 30 Gew.% Chrom, 5 bis 15 und vorzugsweise 5 bis 8 Gew.% Aluminium und 0 bis 5 und vorzugsweise 0 bis 3 Gew.% Molybdän legierter Stahl thermisch auf die Oberfläche des zu beschichtenden Teils gespritzt wird, das Chrom und Aluminium während des Beschichtungsverfahrens in der Spritzmasse (dem Spray) oxidieren, wodurch Chrom- und Aluminiumoxide gebildet werden, die von einer Stahlmatrix umgeben im Inneren der Beschichtung verbleiben, und die Oberfläche der so gebildeten Beschichtungsschicht der Oxidationswirkung der Luft ausgesetzt wird, um einen dichten Chrom- und Aluminiumoxidfilm zu bilden.

4. Verfahren nach Anspruch 3, bei dem eine Schicht mit einer Dicke von 0,3 bis 2,5 mm gebildet wird.

5. Verfahren nach Anspruch 3 oder 4, bei dem das thermische Spritzen nach dem Lichtbogen-, Plasma- oder Ultraschallverfahren durchgeführt wird.

## Revendications

1. Revêtement sur une pièce d'acier utilisable pour protéger le carter, les surfaces de séparation, la tuyauterie, les surchauffeurs et d'autres pièces d'acier d'une turbine à vapeur qui sont soumises, dans une installation de turbine, à une certaine usure par corrosion et érosion, provoquée par la vapeur saturée chaude, qui peut être obtenue en pulvérisant thermiquement un acier allié avec 20 % à 45 %, et de préférence 22 % à 30 % en poids de chrome, 5 % à 15 %, et de préférence 5 % à 8 % en poids d'aluminium, et à 0 % à 5 %, et de préférence 0 % à 3 % en poids de molybdène sur la surface de la pièce à revêtir, le chrome et l'aluminium s'oxydant dans le jet de pulvérisation au cours de l'opération de revêtement, de sorte qu'il se forme des oxydes de chrome et d'aluminium qui resteront dans le revêtement, entourés par une matrice d'acier, et en exposant la surface de la couche de revêtement ainsi formée à l'effet oxydant de l'air pour former un film dense d'oxyde de chrome et d'aluminium.

2. Revêtement selon la revendication 1, constitué d'une couche d'une épaisseur de 0,3 à 2,5 mm

3. Procédé de revêtement du carter, des surfaces de séparation, de la tuyauterie, des surchauffeurs et d'autres pièces d'acier d'une turbine à vapeur qui sont soumises, dans une installation de turbine, à une certaine usure par corrosion et érosion causée par la vapeur saturée chaude, dans lequel un acier allié avec 20 % à 45 %, et de préférence 22 % à 30 % en poids de chrome, 5 % à 15 %, et de préférence 5 % à 8 % en poids d'aluminium, et 0 % à 5 %, et de préférence 0 % à 3 % en poids de molybdène est pulvérisé thermiquement sur la surface de la pièce à revêtir, le chrome et l'aluminium s'oxydant dans le jet de pulvérisation au cours de l'opération de pulvérisation, de sorte qu'il se forme des oxydes de chrome et d'aluminium qui resteront à l'intérieur du revêtement, entourés d'une matrice d'acier, et dans lequel la surface de la couche de revêtement ainsi formée est exposée à l'effet oxydant de l'air pour former un film dense d'oxyde de chrome et d'aluminium.

4. Procédé selon la revendication 3 dans lequel la couche est formée avec une épaisseur de 0,3 à 2,5 mm.

5. Procédé selon la revendication 3 dans lequel la pulvérisation thermique est conduite par une technique d'arc, de plasma ou supersonique.
